

# UNITED STATES PATENT OFFICE.

JOHN B. FIDLAR, OF THE UNITED STATES ARMY.

## PROPELLENT POWDER TO BE USED IN GUNS AND HOWITZERS.

No Drawing.

Application filed December 5, 1921. Serial No. 520,131.

(FILED UNDER THE ACT OF MARCH 3, 1883, 22 STAT. L., 625.)

*To all whom it may concern:*

Be it known that I, JOHN B. FIDLAR, captain, Ordnance Department, U. S. Army, a citizen of the United States, stationed at Picatinny Arsenal, Dover, New Jersey, have invented an Improvement in Propellant Powder to be Used in Guns and Howitzers, of which the following is a specification.

The invention described herein may be used by the Government, or any of its officers or employees in prosecution of work for the Government, or by any other person in the United States, without payment to me of any royalty thereon.

The subject of this invention is a propellant powder to be used in guns and howitzers.

The main object of the invention is the production of a flashless non-hygrosopic propellant powder which may be produced in the form of a single or multi-perforated cylinder, similar to the present form of canon powder grain.

In carrying out my invention I combine a nitrocellulose with a flame reducing ingredient such as starch and overcome the hygroscopic features introduced into the

powder by the starch by the use of nitrohydrocarbon, for example, dinitrotoluene, and to the composition may be added, if desired, a stabilizing reagent, for example, diphenylamine.

A preferred mixture is given by way of illustration and consists of:

Nitrocellulose, 80 plus or minus 10 parts.

Starch, 10 plus or minus 5 parts.

Dinitrotoluene, 10 plus or minus 5 parts.

Diphenylamine, 0.5 plus or minus 0.5 parts.

I claim—

1. A propellant powder, comprising nitrocellulose, starch, dinitrotoluene and diphenylamine.

2. A propellant powder, comprising nitrocellulose, starch and dinitrotoluene.

3. A propellant powder comprising nitrocellulose, a flame reducing ingredient and a nitrohydrocarbon capable of reducing hygroscopicity.

4. A propellant powder comprising nitrocellulose, a flame reducing ingredient, a nitrohydrocarbon capable of reducing hygroscopicity and diphenylamine.

JOHN B. FIDLAR.